

July 1, 1941.

W. J. CHAMPION

2,247,349

BRIGHT COPY HECTOGRAPH DUPLICATION

Filed April 13, 1940

*Fig. 1.*



*Fig. 2.*



*Inventor:*  
By: William J. Champion  
Zabel, Carlson, Dutzbach & Wells  
Attorneys

## UNITED STATES PATENT OFFICE

2,247,349

## BRIGHT COPY HECTOGRAPH DUPLICATION

William J. Champion, Berwyn, Ill., assignor to  
 Ditto, Incorporated, Chicago, Ill., a corporation  
 of West Virginia

Application April 13, 1940, Serial No. 329,429

12 Claims. (Cl. 41—31.6)

The invention relates to hectographic duplicating and has particular reference to means for and methods of producing extremely bright copies.

A primary object of the invention is to provide a duplicating pad or roll having a copy mass which gives extremely bright copies and which has very low adhesion to paper. The low adhesion to paper is desirable because it leads to considerably improved running properties and eliminates sticking of the paper to the copy mass, burning of the roll, and similar undesirable effects.

Most means for increasing copying strength depend on softening the copy mass or increasing the tackiness of the mass, which in turn leads to impaired running properties. The copy brightening means contemplated in this invention do not have these drawbacks.

I have discovered that high copying strength with improved running qualities are obtained if an alkyd resin is incorporated in the gelatinous hectograph copy mass.

Other objects and advantages of the invention will become apparent as the following detailed description progresses, reference being had to the accompanying drawing wherein—

Fig. 1 is a sectional elevation of a hectograph pad constituting a preferred embodiment of the invention;

Fig. 2 is a sectional elevation of a modified hectograph pad.

In Fig. 1, the reference character 1 designates a gelatinous composition containing an alkyd resin uniformly dispersed therein forming the copy mass which is secured to a backing 3 of paper, cloth or other suitable material, by means of a bonding layer 2 which may be of any of the usual compositions such as linseed oil, fish oil, or lacquers containing tanning agents or wetting agents or other suitable bonding agents which have been used to obtain increased adhesion of a copy mass to a backing.

The bonding layer is not essential but is very desirable for hectograph rolls. A hectograph pad which does not have an intermediate bonding layer is shown in Fig. 2 wherein the reference numeral 1 represents the gelatin-alkyd resin composition secured directly to the backing 3.

The copy mass embodied in the present invention comprises a gelling agent such as glue or gelatin; water; a softener such as glycerin, invert sugar, sodium lactate or the like; preferably a hardener such as formaldehyde or other

protein precipitant, and an alkyd resin uniformly dispersed in the mixture.

In one embodiment of the invention, auxiliary color intensifiers are used with the alkyd resin in the gelatinous copy mass. Highly suitable substances are ethylene glycol, diethylene glycol, and sorbitol, which preferably are used in small amounts such as from  $\frac{1}{2}$  to 3%. Also with less satisfactory results but with some advantage in copying qualities there may be incorporated small proportions of diethylene glycol monoethyl ether, diethylene glycol monobutyl ether, and dimethoxytetra glycol. In small amounts these substances have a dye intensifying action which is due to something more than solvent action as shown by the fact that sorbitol, emulsified oil, greases and waxes, which are poor solvents or non-solvents for hectograph dyes also increase the color intensity.

The alkyd resin, preferably in a fluid state is mixed with the gelatin, water and other ingredients and heated in a water bath with stirring until the gelatin dissolves and the ingredients are uniformly dispersed so that they will not settle out on standing. The fluid composition so formed is then coated on the backing and allowed to gel, forming a hectograph blanket.

It is not necessary to incorporate the alkyd resin as such in the mixture. For example, phthalic anhydride may be incorporated in a duplication mass which comprises gelatin, water and glycerin. In this case the phthalic anhydride or phthalic acid in the mass will react with the glycerin forming sufficient alkyd resin to give the desired effect. It appears, however, that even prior to reaction of the polyhydric alcohol with the polybasic acid there is attained some advantage in increased color brightness from the copy mass.

The alkyd resins contemplated include all the resinous (fluid or solid) reaction products of polyhydric alcohols with polybasic acids such as are obtained by reaction between glycerin, ethylene glycol, diethylene glycol, sorbitol, and the like, with phthalic anhydride (or acid), succinic acid, maleic acid, and the like. It is intended to include in the term "alkyd resin" the alkyl phthalyl alkyl glycolates known as "Santicizers." Suitable alkyd resins are also the modified alkyd resins such as cottonseed oil, modified glycerol phthalate resins, and glycerol phthalate resins modified with fatty acids. It is advisable to use alkyd resins which are wholly or partially compatible with the gelatin, water and glycerin of the hectograph composition.

To illustrate the invention, the following formulae of suitable hectograph compositions are given:

|                             | Fairly bright copies | Medium bright copies | Very bright copies |
|-----------------------------|----------------------|----------------------|--------------------|
|                             | Per cent             | Per cent             | Per cent           |
| Glycerol phthalate resin    | 0.25                 | 1.0                  | 5.0                |
| Gelatin, bloom strength 220 | 7.00                 | 7.0                  | 7.0                |
| Water                       | 10.00                | 10.0                 | 10.0               |
| Glycerin                    | 82.75                | 82.0                 | 78.0               |

As an example of glycerol phthalate resins which are suitable in the above composition, the following are given:

(1) *Phthalic glyceride resin*

|                                 | Grams |
|---------------------------------|-------|
| Glycerin                        | 100   |
| Phthalic anhydride              | 160   |
| Acetamide (catalyst)            | 5     |
| Heat 210° C. for one-half hour. |       |

(2) *Stearic phthalic glyceride*

|                               | Grams |
|-------------------------------|-------|
| Stearic acid                  | 60    |
| Phthalic anhydride            | 160   |
| Glycerin                      | 100   |
| Heat one-half hour at 210° C. |       |

(3) *Oleic phthalic glyceride*

|                               | Grams |
|-------------------------------|-------|
| Oleic acid                    | 60    |
| Phthalic anhydride            | 160   |
| Glycerin                      | 100   |
| Heat one-half hour at 210° C. |       |

The above resins are fluids and form opalescent mixtures with the gelatin-water-glycerin. They appear to be dispersed in the composition in the form of particles of colloidal dimensions. However, I do not intend to be limited as to the manner in which the alkyd resin is dispersed in the hectograph composition.

Alkyd resin plasticizers, which are in some measure miscible or soluble with glycerin but still not sufficiently soluble therein to form a true solution, will cause the desired copy brightness, without inducing the excessive "sweating." As examples of these substances may be mentioned the santicizer group of plasticizers, and in particular ethyl phthalyl ethyl glycolate and butyl phthalyl butyl glycolate. These ingredients may be used to advantage in percentages between 2% and 7% of the total weight of the composition but generally I prefer to use about 1 to 3 per cent, as this amount of the ingredient appears to give the most advantageous brightening effect; if the amount of copy brightening agent exceeds about 7 per cent, the mass will tend to become too soft and even sticky, and might show an objectionable solvent action toward the lacquer in the roll backing. However, this may be compensated for by increasing the glue or gelatin content of the roll and then amounts even higher than 7 per cent may be employed.

In order to counteract any tendency for attacking the lacquer on the roll backing, I may incorporate with the brightening agent materials soluble in the brightening agent but not solvents for lacquer. I may mix with the brightening agent a proportion of glycol or glycerol esters or the like, or of mineral oil.

The following examples illustrate the invention:

*Example I*

|                                            | Parts |
|--------------------------------------------|-------|
| 5 Gelatin                                  | 30    |
| Water                                      | 45    |
| Glycerin                                   | 360   |
| Ethyl phthalyl ethyl glycolate (by weight) | 8     |

*Example II*

|                                | Parts |
|--------------------------------|-------|
| Gelatin                        | 30    |
| Water                          | 45    |
| Ethyl phthalyl ethyl glycolate | 2     |
| Chrome alum                    | 15    |
| Glycerin                       | 400   |

*Example III*

|                                | Parts |
|--------------------------------|-------|
| Glue                           | 60    |
| Water                          | 90    |
| Glycerin                       | 350   |
| Sorbitol                       | 10    |
| Chrome alum                    | 15    |
| Formaldehyde                   | 15    |
| Butyl phthalyl butyl glycolate | 12    |

*Example IV*

|                                | Parts |
|--------------------------------|-------|
| Glue                           | 60    |
| Water                          | 90    |
| Glycerin                       | 400   |
| Butyl phthalyl butyl glycolate | 10    |
| Diglycol oleate                | 2     |

These examples have been given by way of illustration only and should in no sense be construed as limitations.

Copies are prepared from the hectograph pad of the invention in the usual manner. A design is formed on a copy paper by writing or typing with a hectograph ink made of a water or alcohol soluble dye such as methyl violet, crystal violet, fuchsin and the like. The design is then contacted with the gelatinous copy surface of the pad, whereupon the dye is largely transferred to the composition giving the design in mirror reverse. Copies are then made by contacting sheets of paper with the design on the hectograph copy mass. It will be found that a large number of copies of high color intensity can be obtained when the gelatinous copy mass contains a polyhydric alcohol and a polybasic acid, particularly when these ingredients have combined to form the alkyd resin.

While I have shown and described certain embodiments of my invention, it is to be understood that it is capable of many modifications. Substitutions of equivalent materials and changes in the proportions may be made without departing from the spirit and scope of the invention as described in the appended claims in which it is my intention to claim all novelty inherent in my invention as broadly as possible in view of the prior art.

I claim:

1. A hectograph blanket comprising a gelatinous copy mass containing a polyhydric alcohol and a polybasic acid.
2. A hectograph blanket comprising a gelatinous copy mass containing an alkyd resin.
3. A hectograph blanket comprising a copy mass containing gelatin, water, glycerin and an alkyd resin.
4. A hectograph blanket comprising a copy mass containing gelatin, water, glycerin, an alkyd resin, and a substance selected from a group

consisting of glycols, glycol ethers, sorbitol and emulsified oils, waxes, and fats.

5. A hectograph blanket comprising a copy mass containing gelatin, water, glycerin, an alkyd resin, and a minor proportion of ethylene glycol. 5

6. A copy mass comprising gelatin, water, a polyhydric alcohol, and a polybasic acid.

7. A copy mass comprising gelatin, water, glycerin, and an alkyd resin.

8. A copy mass comprising gelatin, water, glycerin, an alkyd resin, and a substance selected from the group consisting of glycols, glycol ethers, sorbitol, and emulsified oils, waxes, and fats.

9. A copy mass comprising gelatin, water, glycerin, an alkyd resin, and a minor amount of 15 ethylene glycol.

10. A composition particularly adapted for

hectograph copy masses comprising gelatin, water, a polyhydric alcohol and a polybasic acid.

11. A composition particularly adapted for hectograph copy masses comprising gelatin, glycerin, a polybasic acid, and a substance selected from the group consisting of glycols, glycol ethers, sorbitol, and emulsified oils, waxes, and fats.

12. The method of producing copies of high color intensity which comprises contacting a sheet having a design of a water and alcohol soluble basic dye with a gelatinous copy mass containing an alkyd resin whereupon the design in reverse appears upon the copy mass, and contacting the design on the copy mass with a copy sheet to transfer the design to the copy sheet.

WILLIAM J. CHAMPION.